

## UNITED STATES PATENT OFFICE

2,244,363

## METHOD OF MAKING YARN

Clifford Holdsworth, Sanford, Maine, assignor to  
 Goodall Worsted Company, Sanford, Maine, a  
 corporation of Maine

No Drawing. Application August 2, 1940,  
 Serial No. 350,107

1 Claim. (Cl. 57—156)

This invention relates to the manufacture of yarn made from the Angora fleece, and it has for its object to provide a novel method by which a yarn can be made that contains all the fibres of the fleece regardless of their length or character. It has been found that a yarn made in accordance with this invention is smooth, free from slubbings and has increased elastic qualities which make for easier weaving.

In making mohair yarn from the fibres of the Angora fleece, it has heretofore been customary to first sort the fibres of each fleece into different grades or "sorts," one grade comprising generally the long fibres, another grade comprising the shortest fibres, another grade comprising the coarse fibres, another grade comprising the fine fibres, etc. Usually the fleeces are sorted into seven or more grades or sorts.

After sorting the fibres of the fleece, then each grade or "sort" is subjected separately to the various operations, such as scouring, carding, card gilling, combing, gilling, drafting and spinning, etc., to which fibres are usually subjected when converting fibres into yarn.

In accordance with this invention, the operation of "sorting" the fleece is dispensed with and all the fibres of the fleece are kept together while being subjected to the carding, card gilling, drafting, spinning, and other operations involved in converting the fibres into yarn. At every stage of the new method, the sliver or roving is one that contains all the fibres of the fleece whether they be long or short, or coarse or fine, or stiff or silky, the fibres of various types being mixed together in the sliver, roving or yarn in the same proportions that they are to be found in the fleece.

In practicing the present invention, the unsorted Angora fleece is first dusted and scoured, these operations being carried out in the usual manner, although it has been found that it is preferable to run the fleece through the duster twice, as the double dusting opens up the fibres better and shakes out more dust and dirt. If the fleece contains any badly stained fibres, it is well to remove them before the dusting operation, but nothing is done in the way of sorting or grading the fibres.

After the dusting and scouring operations, the fibrous mass, which contains all the fibres of various kinds found in the original fleece and in the same proportions as in said fleece, is subjected to a carding operation to straighten the fibres and lay them more or less parallel. Such carding operation is carried out in the usual way

and by usual means except that the carding machine is so adjusted that the sliver comes off approximately 40% smaller than usual. The doffer roll is also speeded up so that there will be the same production in spite of the fact that the sliver is smaller.

After the carding operation, the fibre mass is subjected to the card gilling operation which is the same as usual except that instead of feeding 6 to 8 ends to the gill box, as is done when treating sorted fibres, 8 to 12 ends are fed in simultaneously. Since the ends are smaller by 40%, the addition of the greater number of ends makes up the requisite quantity. The gill boxes are also set closer, the spacing between the fallers and each of the front rolls and back rolls being reduced about one half an inch for the first gill box and about one half that for the second gill box. The sliver which is delivered from the gill boxes is about 10% smaller than normal. In the second gill box, 8 ends are fed in simultaneously, instead of the usual 6 ends, thus making a 33 1/3% increase.

The usual operation of combing after the card gilling is entirely omitted, and from the second gill box the sliver containing all the various lengths and types of fibre found in the original fleece goes directly to the finish gilling.

Since it is the purpose of this new method to produce a yarn containing all of the fibres of Angora fleece, both short and long, coarse and fine, the use of the Noble combor would defeat this purpose, as it would remove the short fibres.

In feeding the sliver to the finish gilling, about 10% more ends are fed into the back gill box to make up for the 10% smaller size of the sliver, and both the back gill box and the front gill box have closer settings to enable them to handle the fibre mass containing the short fibres as well as the long fibres. From the finish gilling, the balls of sliver containing all the fibres of the original fleece go to the drafting department, as usual. The first operation in this department is on the so-called "two-spindle gill box" which puts the sliver on a large wooden spool, at which time it is known as a slubbing. In this two-spindle gill box, four ends are fed in at the same time instead of three, as is the practice in treating slivers of sorted fibre, and the slubbing comes out about 10% smaller than normal. The settings of the two-spindle gill box are also slightly reduced.

From then on through the five drawing operations there is no increase in doublings, but each drafting apparatus has closer settings than normal. On the last of the heavy drawing opera-

tions the doublings are increased 25% to make up for the 10% reduction in size of the slubbing. The slubbing as it comes from the last heavy drawing operation is about 15% smaller than normal. It then goes to the rover where two ends instead of one are fed in, and extra draft is given to reduce the doubled slubbing to normal size. Furthermore, the settings are closer, and steel carrier rolls are used instead of the wooden carrier rolls. The steel rolls give sufficient weight 10 to hold the short fibres and control the drawing thereof, but not sufficient weight to cause breakage of the long fibres. A small top front roll is used and the front carrier roll is set as close as possible to the front rolls. The builder motion is 15 preferably adjusted to relieve the tension on the short fibres, and is slowed down and arranged so that the roving is wound on the spool in close coils rather than in coarse coils.

After the drafting operation, the roving, which 20 contains all the fibres of various lengths and kinds that are present in the original Angora fleece, and in the same proportions as existed in such fleece, is subjected to the spinning operation to convert the roving into yarn. This spinning operation is carried out on any usual spinning apparatus, except that two rovings instead of one are fed into the machine and an increased draft is produced in order to secure yarn of the proper count. The settings of the rolls are also 25 closer. The back roll and front roll are set about one-half inch longer than the longest fibre, but the carrier rolls are set very close to the front roll.

A single ply yarn is thereby produced which is 30 smooth, free from slubbings, and contains all the fibres of the Angora fleece, long fibre, short fibre,

medium length fibre, fine fibre, coarse fibre, etc., and in approximately the same proportions as exist in such fleece. The yarn has increased elastic qualities and, therefore, is easier to use in weaving operation.

5 I claim:

The method of making from the Angora fleece yarn which contains all the various kinds and lengths of fibres existing in the fleece and in substantially the same proportions as found in the fleece, which method consists in subjecting the unsorted fleece containing all its original fibres to a carding operation by which a sliver is produced containing fibres of all the various lengths and types found in the original fleece but approximately 40% smaller than normal, subjecting this sliver to a card-gilling operation in which a sufficiently greater number of ends than normal is fed into the gill-box to compensate for the subnormal size of the sliver, transferring the sliver from the gilling operation directly to a finish gill box having closer settings than normal and in so doing feeding extra ends to the back gill-box to make up for the smaller size of the sliver, subjecting the sliver containing fibres of all the various lengths and types found in the original fleece to the usual plurality of drafting operations in drafting apparatus having closer settings than normal and provided with carrier rolls of sufficient weight to hold the short fibres but of insufficient weight to break the long fibres, thereby converting the sliver into a roving containing fibres of all the various lengths and types found in the original fleece, and then spinning the roving into a single ply yarn.

CLIFFORD HOLDSWORTH.